

Nov. 15, 1932.

L. ALLEN ET AL

1,888,154

MANUFACTURE AND PRODUCTION OF TRANSFERS

Filed Oct. 19, 1928

Fig. 1.



Fig. 2.



Fig. 3.



Fig. 4.



INVENTORS

LEONARD ALLEN  
ERNEST CHARLES DEERING  
by his attorneys.

Howson and Howson

Patented Nov. 15, 1932

1,888,154

# UNITED STATES PATENT OFFICE

LEONARD ALLEN, OF BURSLEM, AND ERNEST CHARLES DEERING, OF NEW BARNET,  
BARNET, ENGLAND

## MANUFACTURE AND PRODUCTION OF TRANSFERS

Application filed October 19, 1928, Serial No. 313,641, and in Great Britain March 16, 1928.

This invention relates to printing lustre or "liquid metal" transfers, which may or may not be combined with colors, on paper by means of letter press, copper plate, or 5 other printing processes, and subsequently applying the transfers to pottery, glass, enamelled iron, jewellery or the like.

In the drawing Fig. 1 is a broken perspective view of a simplex paper with a transfer 10 impressed thereon according to our invention.

Fig. 2 is a longitudinal cross section view of the combination shown in Figure 1.

Fig. 3 is a broken perspective view of a 15 duplex paper with a transfer impressed thereon.

Fig. 4 is a longitudinal cross section view of the combination shown in Fig. 3.

In carrying out our invention the transfers 20, which may be of "liquid metal" or lustre, are printed upon either simplex or duplex paper, as shown in the drawing. These papers are well known in the art. In the case of the simplex paper shown in Figs. 25 1 and 2, the paper consists of ordinary paper 1, having a glazed surface 2, upon which the transfers may be impressed by known printing processes such as letter press, offset, copper plate, or the like. In the case of duplex paper, shown in Figures 3 and 4, the paper consists of ordinary paper 1 upon 30 which is superimposed tissue paper 4 coated so as to have a glazed surface 5 upon which the transfers may be impressed in the same way as with simplex paper. The glazes 2 and 5 may be of vegetable or any other size 35 that is usually found on commercial transfer papers. The composition of these glazes is optional and forms no part of the present invention.

If desired, colors 6 may be combined with the "liquid metal" or lustre transfers. If colors are to be used two or more superimposed registering impressions may be made 45 so as to produce the sufficient body in the print.

The "liquid metal" hereinbefore referred to is well known in the art and consists of metals such as silver, gold or the like which 50 after having been finely divided are dis-

solved or suspended in essential oils. If desired these solutions may contain two or more of these metals.

We have found that a single impression is sufficient to yield highly satisfactory transfers if the "liquid metal" or lustre, which contains a high percentage of resinous material is heated to the state where a certain proportion of the volatile oils are driven off and the "liquid metal" or lustre becomes 55 more or less permanently tacky and approaches the point of decomposition, the resultant product of "liquid metal" or lustre being thus more easily and economically worked both for printing transfers generally 60 by any printing process and in particular for printing in letter press or offset printing and also in copper plate methods. After printing on the paper the film shortly becomes dry 65 and hard.

In order that these transfers may be transferred to pottery, glass, enamelled iron, jewellery or the like used is made of the fact, above stated, that the liquid metal or lustre contains a high percentage of resinous material, which will become tacky at elevated 70 temperatures. To effect transference, the article, or object to be decorated is first slightly moistened and the said transfers are then applied face downwards in the usual manner, when the article or object is suitably heated. The paper with its adhesive coating 75 is subsequently removed by washing or by any convenient method with or without cooling.

The following examples further serve to illustrate how the transference may be effected onto the articles or bodies to be decorated.

### Example 1

The article to be decorated is slightly moistened and the transfer is applied, when the article is heated to about 50° to 70° Centigrade. After cooling, the paper with its 95 adhesive coating, is removed by washing with water.

### Example 2

The article to be decorated is heated to about 50° to 70° Centigrade, and the transfer is applied.

are then applied and after cooling, the paper is removed followed by washing in the usual way as described in Example 1.

*Example 3*

5 The article is moistened with warm water, the transfer applied and the paper removed, followed by washing as already described.

*Example 4*

10 The article is moistened and the transfer applied and pressed down by rubbing with a hot dry cloth; the paper is then removed followed by washing as already described.

15 Ordinary ceramic colour transfers, as now made may have additional details in liquid metals or lustres added, and the transfers so treated are transferred by the methods we have described. As however these methods of transference are not entirely satisfactory 20 as regards the colour portions 6, one of the following alternative methods may be adopted according to this invention which yield very satisfactory results.

25 The colour portion only on the transfer is printed or painted over with a thin film 7 of resinous material for example a solution of resin in a volatile oil and the transference is then carried out according to one of the methods already described.

30 Alternatively instead of printing the colour transfer by employing an oil or fatty medium with the colour, the medium used is a solution of a resinous material which introduces 35 the required resin for the transference and the transfers can then be printed for example in a letter press or offset machine or from a copper plate and perfect transference can thus be obtained with mixed metal, lustre 40 and colour transfers.

45 When transfers are printed on duplex paper the upper and thinner surface portion of the paper with the transfer thereon is stripped from the under or heavier portion 50 of the paper before applying the transfer to the body to be decorated.

55 It will be understood that the adhesive coating to be removed from the article after the application of the transfer is that contained on the ordinary duplex or simplex transfer paper, but in order to obtain the most satisfactory results from the point of view of brilliancy with "liquid metal" or lustre transfers we preferably use a specially prepared transfer paper in which the amount of adhesive coating used is reduced to a minimum. This is of special value as an aid to the application of the transfers to curved surfaces, while on practically flat surfaces 60 the adhesive coating may be entirely dispensed with, a surface hardened paper being used in order to obtain a good print for transference. After transference the article may be fired, as is customary in the art, to fix the 65 transfers, but this step forms no part of the

present invention and therefore we do not claim it.

What we claim is:—

1. The manufacture of transfers for decoration of articles having a smooth, glass-like 70 surface, comprising printing transfers of finely divided metals in essential oils, upon transfer paper.

2. The manufacture of transfers for decoration of articles having a smooth, glass-like 75 surface, comprising printing transfers of finely divided metals in essential oils, upon transfer paper having a minimum amount of adhesive coating thereon.

3. The manufacture of transfers for decoration of articles having a smooth, glass-like 80 surface, comprising heating a quantity of finely divided metal which has been mixed with essential oils, to a point whereat the substance becomes tacky and readily usable 85 in a printing press and after printing will adhere to articles merely upon the application of a low degree of heat, and printing with said heated mixture upon a transfer paper.

4. The manufacture and production of transfers, for decoration of articles having a smooth glassy surface, comprising heating finely divided metals in essential oils, to a point whereat the mixture becomes tacky, subsequently printing with such mixture upon transfer paper, printing color transfers on said paper, and painting over said colors with a film of resinous material prior to effecting transfers from the paper to the article to be decorated.

In testimony whereof we have signed our names to this specification.

LEONARD ALLEN.

ERNEST CHARLES DEERING.

105

110

115

120

125

130